

E. E. NOVOTNY,  
LITHOGRAPHIC AND OFFSET PRINTING PLATE,  
APPLICATION FILED DEC. 30, 1916.

1,357,340.

Patented Nov. 2, 1920.

2 SHEETS—SHEET 1.

*Fig. 1.*



*Fig. 2.*



*Fig. 3.*



*Fig. 4.*



*Fig. 5.*



*Fig. 6.*



*Fig. 7.*



Inventor,  
*Emil E. Novotny.*

By his Attorneys,

*Meyers, Cushman & Keen*

E. E. NOVOTNY.  
LITHOGRAPHIC AND OFFSET PRINTING PLATE.  
APPLICATION FILED DEC. 30, 1916.

1,357,340.

Patented Nov. 2, 1920.

2 SHEETS—SHEET 2.



Fig. 9.



Fig. 10.



Fig. 11.



Fig. 12.



Inventor,  
Emil E. Novotny.

By his Attorneys,

Meyers, Cushing & Rea

# UNITED STATES PATENT OFFICE.

EMIL E. NOVOTNY, OF RIVERSIDE, ILLINOIS, ASSIGNOR TO J. STOGDELL STOKES, OF MOORESTOWN, NEW JERSEY.

## LITHOGRAPHIC AND OFFSET PRINTING PLATE.

1,357,340.

Specification of Letters Patent.

Patented Nov. 2, 1920.

Application filed December 30, 1916. Serial No. 139,721.

To all whom it may concern:

Be it known that I, EMIL E. NOVOTNY, a citizen of the United States, residing at Riverside, in the county of Cook and State of Illinois, have invented certain new and useful Improvements in Lithographic and Offset Printing Plates, of which the following is a specification.

This invention relates to a printing plate 10 which is particularly adapted for use in connection with various printing processes, such as lithographic, offset printing and planographic work in general.

In the present instance it is my purpose to 15 provide a printing plate which is formed of a material or materials capable of being molded or shaped to any desired form or dimensions and having a face which is susceptible of treatment to produce a surface 20 for the practice of printing processes such as those above mentioned. To accomplish this I have produced a plate which embodies or includes a body of plastic material such as a phenolic condensation product having combined therewith, preferably in granular or powdered form, a suitable substance, such as lithographic stone or metal, depending upon the purpose for which the plate is to be employed. Such a plate may be made of 25 any desired shape or contour, either flat, curved or cylindrical and may be either flexible or inflexible in its nature. In this connection I wish to state that I realize that the invention in its broad aspects may be 30 embodied in various forms, and therefore, while I have herein shown and described a preferred embodiment of the invention, as well as certain chosen modifications thereof, I wish it to be understood that I do not limit 35 myself to these particular exemplifications, as modification and variation may be made without departing from the spirit of the invention or exceeding the scope of the appended claims.

40 My invention consists in the printing plate and the method of making the same set forth in and falling within the scope of the appended claims.

In the accompanying drawings:

45 Figure 1 is a conventional view of a press and showing a plate being molded therein.

Figs. 2 to 7 inclusive are detail views 50 showing plates embodying my invention wherein the printing surface of each of the plates is made of a coating of powdered ma-

terial united with a backing layer of plastic material.

Fig. 8 is a detail view partly in section showing a segmental form of plate mounted on a press cylinder, the printing surface of 60 the plate being also in the nature of a coating of powdered material.

Figs. 9 and 10 are end views showing cylindrical plates mounted on press arbors or cylinders, the printing surfaces of these 65 plates being also formed of powdered material.

Fig. 11 is a cross sectional view of a modified form of flat plate, in this instance the powdered material being incorporated in the 70 body of plastic material.

Fig. 12 is a similar view, but showing a cylindrical plate wherein the powdered material is incorporated in the plastic material.

As is well known, at the present time, in 75 lithography the printing plate is composed of either a lithographic stone or of a metal such as zinc or aluminum. The lithographic stone plate possesses certain advantages due primarily to its inherent porosity which enables it to readily hold the grease, retain the water, and take on the desired grain. On the other hand, such a stone plate is naturally restricted in its use to a flat form 80 usable on a flat bed press, and is therefore, 85 not adapted for use in conjunction with a high speed rotary press. Furthermore, after such a stone has been used for the printing of a particular design, work or image, and it is desired to remove the latter from the stone 90 in order to apply another design, work or image to the face of such stone, it is necessary to follow out a tedious process of cleaning and polishing the stone surface, this work requiring considerable care and necessitating the employment of an expert. Of course the frequent re-polishing and re-graining of the stone naturally reduces its 95 thickness and in the course of time such stone must be discarded.

100 Metallic plates used in lithography, such as those composed of zinc or aluminum, possess the advantage that they may be employed on rotary presses, due to the inherent flexibility of the thin metallic plate which enables it to be bent into form to be applied to the curved surface of the cylinder. However, such a metallic plate is incapable of 105 taking on the fine printing surface of a desired grain, which is attainable with the 110

- lithographic stone, and furthermore, such metallic plate requires considerable expert work in the production of the grain for the printing surface because the metal is not sufficiently porous in its nature, and consequently even when the greatest of care is exercised in the preparation of the plate the moisture-retaining qualities of the grain is inferior to that of the lithographic stone.
- 10 Thus, while it is possible to print directly on the paper from a lithographic stone when the latter is resting on its flat bed, it is the present practice to use the metal lithographic plate in doing offset work, that is to say, the image, work or design appearing on the metal plate is first transferred to an offset roller of rubber, and then such offset roller acts directly upon the paper to transfer the design, work or image to the latter.
- 15 20 As contradistinguished from the lithographic stone and from the metal lithographic plate, I have provided a printing plate which while having inherent therein the advantages of both the above mentioned types of plates it is free from the disadvantages and draw-backs just mentioned as incident to the latter.
- In Figs. 1 to 10 inclusive, I have shown a printing plate which may be used for lithographic, planographic and offset printing and wherein the printing face of the plate is formed of a coating of powdered or granular material united with a backing of plastic material, various forms of supports or bases being shown in the various views. In Figs. 11 and 12 the powdered or granular material instead of being in the form of a coating is intimately commingled or incorporated in the body of plastic material.
- 30 35 40 45 In Fig. 1 I have conventionally illustrated a press for molding the plate and will describe in connection therewith the manufacture of the plate illustrated in Fig. 2.
- Referring to said Figs. 1 and 2, the numeral 1 indicates the bed of the press while 2 is the top platen thereof, and such press is intended to be heated and cooled in any suitable manner. Upon the bed 1 of the press I first place a base 3 which is in the nature of a metal sheet, and is preferably formed with a series of dovetailed apertures 4 therein. On such metal base I impose a sheet 5 of plastic material, preferably in the nature of a phenolic condensation product of which there are a number of well known varieties such as "bakelite" or "condensite." As is well known, such a phenolic condensation product possesses marked advantages from the standpoint of strength, durability, incompressibility and capability of retaining the shape or form to which it has been set. In some of its forms this phenolic material which as is well known is a synthetic resin when completely set assumes a hard, inflexible state and is not thereafter subject to changes even when re-heated. In another form such phenolic material while it may be set or hardened may subsequently be re-heated and re-softened to render it capable of being again worked or flexed as may be desired. I prefer to employ the latter form or grade of the material because while it may be hardened and set by cooling to form a plate of the desired rigidity and unchangeableness of form yet, when the usefulness of the plate for a particular purpose has ended, the phenolic material thereof may be re-heated and re-molded to produce another plate. In other words, such phenolic material may be used and re-used time and again by simply re-heating and re-molding. At the time of imposing the phenolic layer 5 on the metallic base 3, the former is in a relatively soft or plastic stage or condition, of almost putty-like consistency. Pressure is now applied by closing the top platen 2 of the press to smooth or level the phenolic sheet, which also results in forcing some of the phenolic material through the dovetailed apertures or openings 4 of the plate thus forming phenolic lugs 6 which will lock or anchor the layer 5 to the base. At the time of applying this initial pressure, however, the phenolic layer is not compressed or flattened to its final thickness.
- The press is now opened by raising the platen 2 and a coating or layer of powdery substance shown at 7 is now sprinkled or applied to the uppermost face of the plastic material. This granular or powdered material is so applied as to provide a coating or sheet of any desired or required thickness, the amount of the powdered or granular material depending of course upon the dimensions of the plate it is desired to produce, and this may be determined as to thickness by suitable bearers 8 which form a frame on the bed of the press, as will be readily understood. If it is desired to produce a plate having the characteristics of a lithographic stone then the material employed for this top coating 7 is in the nature of pulverized, powdered or granular lithographic stone. Under such conditions the top platen of the press is equipped with a smooth, hard, polished bottom face, such as is shown at 9 so that when the top platen is again closed on the bed of the press this face will contact or press against the layer of granular or pulverized lithographic stone and embed the same in the upper face of the layer of phenolic material, thus facing this phenolic layer with a printing face of stone which when subjected to the action of the etch and gum will readily take on the necessary grain precisely as does the ordinary lithographic stone. When, however, it is desired to form this printing face of the plate of granular metal, the bottom face 9 of the press platen 2 may be grained, so that

when the pressure is applied to embed the metallic particles in the plastic layer, the graining of the bottom face of the platen will be reproduced on the metallic coating 5 or face of the plate thus obviating the necessity of subsequently graining this metallic face to produce the necessary tooth as is required now in the preparation of metallic lithographic plates. Under some conditions 10 it may be desirable to form this printing face or coating 7 of a combination or mixture of powdered or granular metal and lithographic stone or other moisture-retaining substances, such as kaolin, and under 15 these circumstances the subsequent graining of this face, as is required with the ordinary metal plate will not be necessary, as the etch acting on the lithographic stone particles will give the face the necessary tooth or 20 grain and will increase the water retentive qualities of the metallic surface. Of course in employing both the powdered lithographic stone and the granular or powdered metal, care should be taken, to see that these 25 are clean and sensitive before being applied to the plastic or phenolic layer. When this second stage of the making of the plate has been completed through heat, pressure and cooling while such plate is in the press, the 30 press may be opened and the plate removed, such plate having been of course permitted to remain in the press preferably a sufficient length of time to set or harden to an inflexible form. When removed, the plate will 35 appear as shown in Fig. 2. Of course when it is to be used in actual work the face 7 is treated or operated upon in the usual manner. That is to say, the image or work is applied thereto as is ordinarily done with 40 the lithographic stone.

In Fig. 3 instead of anchoring the plastic layer 5 to the base through lugs or openings as is done in Fig. 2, such plastic layer may be cemented directly to the base, or a suitable binder indicated at 10 may be used.

In Fig. 4 the base 3<sup>a</sup> is made of a fibrous material such as compressed paper pulp preferably impregnated with a phenolic material and on this base the plate 5 carrying 50 the powdered face is cemented. If the fibrous plate 3<sup>a</sup> be impregnated with a sufficient amount of the phenolic material it will not be necessary to employ the layer 5, but the powdered facing may be applied directly 55 to the sheet 3<sup>a</sup>.

In Fig. 5 instead of employing a separate base, a plate 5<sup>a</sup> of phenolic material, of suitable thickness is employed and the powdered facing 7 is applied directly to this as before 60 described.

In Fig. 6 a base 3<sup>b</sup> of plastic material has the powdered facing 7 applied thereto, while the opposite face of this base 3<sup>b</sup> is formed with bosses 11 which seat in recesses 12 65 formed on the block support 13, the bosses

and recesses being arranged predetermined and spaced distances apart so that the plate may be positioned and arranged on the support.

In Fig. 7 a metallic back 14 is employed 70 which is in the nature of a shell-like plate having an aperture as at 15 and recesses 16 formed in the upper face thereof, the phenolic layer 17 being applied directly to this face, such phenolic plate 17 75 having bosses 18 molded on the under face thereof which seat in the recesses 16 and having a lug 19 molded through the opening 15. Of course the powdered facing 7 is applied to this phenolic layer 17.

Such a plate as is shown in Fig. 7 may be curved or bowed into segmental form to fit on the cylinder 20 of a press, such cylinder carrying pins 21 which project through recesses 22 in the face of the cylinder, the ends 80 of the pins registering with the perforations 23 in the metallic base 14 of the bed thereby preventing the sliding or shifting of the plate on the cylinder. This cylinder may also have employed in connection therewith magnetic devices 24 which act upon the metallic base 14 of the plate to hold such plate against the cylinder by magnetic attraction.

In Fig. 9 I have shown the plate of cylindrical form, this plate in its component parts being substantially the same as that shown in Fig. 5, that is to say, is formed of a cylinder 24' of plastic material having the face coating 25 of a powdered substance, the complete tubular or cylindrical plate being fitted over a cylinder or arbor 26 forming a part of the press. In this instance the plate may be first made in flat form and then while still warm and capable of being flexed may 95 be rolled into cylindrical shape about a suitable mandrel. Or if desired, the plate shown in Fig. 9 may be cast or molded in cylindrical shape.

In Fig. 10 a metal shell 27 carries the phenolic layer 28, the latter in turn carrying the printing face or coating of the pulverized material, as shown in 29, these being fitted upon the cylinder 30 of the press.

In Fig. 11 the powdered material instead 110 of being applied in the form of a facing coating is intimately commingled with the body of plastic material 31, as is indicated at 32, and in Fig. 12 I have shown a plate of this character made in the form of a 115 cylinder as indicated at 33.

It will be noted that plates embodying my invention may be rapidly and economically produced by exceedingly simple methods and the desired designs may be readily 120 applied to, and when desired, removed from the printing surface of the plate, and furthermore, during the course of its manufacture the plate may be shaped to accommodate itself to any supporting body, such as 130

the cylinder of a printing press. Furthermore, I am enabled to produce plates of any desired contour and hardness or rigidity, and may employ as facings for the plates, 5 or as component parts thereof intimately incorporated therein, any suitable powdered material. The printing faces of my plates may be produced by a simple method of molding with either a highly polished 10 smooth and plane surface of stone, or any desired grain or tooth such as is at present in the art produced by the usual grinding operation. After my plate has been used for the printing of the required number of 15 impressions the printing face thereof may be removed or cleaned by scraping and the plate again re-surfaced with the powdered material and the plate is thus again ready for other and different printing matter if 20 necessary and of a uniform height. Thus I obviate continually reducing or changing the height of the plate, as occurs in the treatment or grinding of the ordinary lithographic stone or metal plate, which as is well 25 known, through successive regrindings finally becomes too thin for practical use and must be discarded.

Another advantage incident to my invention is that I am able to employ a series of 30 my plates on a rotary press or in connection with a rotary offset press or to use any combination of plates on such a press to produce work which resembles either lithographic printing or offset printing. This is made 35 possible through the use of my improved plates which are of uniform thickness or height to paper, of uniform grain and of strong, substantial cross section so that they may be clamped or mounted in any desired 40 interchangeable combinations.

Furthermore, I am enabled to produce on a rotary press work showing greater graduations of tints and full tones than is at 45 present possible in the art due to my printing surface being capable of any desired amount of curvature to form a curved lithographic stone or a metallic surface having incorporated therewith granules or powder

of lithographic stone, kaolin or other water retentive or absorbent materials. This 50 brings in a new field of possibilities in rotary printing as it eliminates the shortcomings of the flexible metallic plate which made rotary planographic printing possible but which depends entirely on the grain or tooth 55 for their water retentive qualities. Furthermore, with this possibility of increased water retentive qualities this plate is capable of printing by direct contact with paper on a rotary type of machine, as is now done in 60 the art with flat, lithographic stone.

What I claim is:

1. A lithographic and offset printing plate comprising a body portion, including a synthetic resinous material, and a printing 65 face for the body portion composed of granular particles and forming a lithographic and offset printing surface bonded to the body portion by the synthetic resinous material.

2. A lithographic and offset printing plate comprising a body portion, including a synthetic resinous material, a toothed printing 75 face for the body portion composed of granular particles and forming a lithographic and offset printing surface bonded to the body portion by the synthetic resinous material, and a backing upon which the body portion is mounted.

3. A lithographic and offset printing plate 80 comprising a fibrous body impregnated with a synthetic resinous material to reinforce such body, and a granular printing face composed of granular particles and forming a lithographic and offset printing surface 85 bonded to the body by the synthetic resinous material.

4. A lithographic and offset printing plate comprising a fibrous body, a granular printing face forming a lithographic and offset 90 printing surface, and a hard and set synthetic resinous material bonding the granular printing face to the fibrous body.

In testimony whereof I affix my signature.

EMIL E. NOVOTNY.